

Dec. 16, 1930.

W. F. BRANDSMA ET AL

1,785,246

MAGNETIC MATERIAL

Filed Aug. 1, 1928

2 Sheets-Sheet 1

*B*=MAGNETIC FLUX

*Fig. 1*



*Fig. 3*



INVENTORS  
W.F. BRANDSMA P.R. DIJKSTERHUIS  
BY G.B. JONAS G.J. SIZOO  
*Mag. J. Adams*  
ATTORNEY

Dec. 16, 1930.

W. F. BRANDSMA ET AL.

1,785,246

## MAGNETIC MATERIAL

Filed Aug. 1, 1928

2 Sheets-Sheet 2



Fig. 2

$$TAN\alpha = \frac{\Delta P}{\Delta H} = \text{EFFECTIVE PERMEABILITY}$$

**INVENTORS**  
W.F. BRANDSMA P.R. DIJKSTERHUIS  
BY C.B. JONAS G.J. SIZOO  
*Sam & Edouard*

*Graff Adams*  
ATTORNEY

## UNITED STATES PATENT OFFICE

WIEBOLD FRANS BRANDSMA, POPKO REINDER DIJKSTERHUIS, GERARDUS JOHANNES SIZOO, AND GOTTFRIED BRUNO JONAS, OF EINDHOVEN, NETHERLANDS, ASSIGNEES TO RADIO CORPORATION OF AMERICA, A CORPORATION OF DELAWARE

## MAGNETIC MATERIAL

Application filed August 1, 1928, Serial No. 296,665, and in the Netherlands July 19, 1927.

This invention has reference to a magnetic material. As is well known in practice, it is possible by special heat operations to exercise a great influence on the properties of 5 magnetic material. When, for example, the material has been decarbonized by heat in air or oxygen, it will be found on experimentation that the permeability has increased. Consequently, it is apparent from 10 the hysteresis curve of the material thus produced that at small values of the intensity  $H$  of the magnetic field the curve ascends steeply and then passes rather sharply into the zone of saturation.

15 Let it be assumed that this material is used as the core of a low-frequency transformer and that this transformer is connected in an amplifying stage of a receiver unit for radio-telephony. To the direct current 20 corresponds a certain field intensity  $H$  and to the alternating current a cyclically varying field intensity  $\Delta H$ . Now, the variations in the flux  $B$  are measured and the coefficient of the maximum  $\Delta B$  and the 25 maximum  $\Delta H$ , i. e.

$$\frac{\text{maximum } \Delta B}{\text{maximum } \Delta H}$$

is determined.

30 These measurements at different values of  $H$  show that the coefficient

$$\frac{\text{maximum } \Delta B}{\text{maximum } \Delta H}$$

35 hereinafter referred to as "effective permeability", depends greatly on the various intensities of field  $H$  at which the cyclically varying  $\Delta H$  occurs. Another fact that is distinctly pronounced during the measuring 40 operations is that the effective permeability depends greatly on the value of the  $\Delta H$  and consequently on the amplitude of the alternating current. It is desirable that this phenomenon should not occur and that the 45 effective permeability at different values of  $H$  should have large and practically constant values. The invention has for its object to so work the material that this requirement is met.

50 According to the invention the previously

decarbonized magnetic material is subjected to a final operation in which the material partly oxidizes. This may be carried out expediently by essentially decarbonizing the material by heat in air or oxygen and then 55 continuing this heating operation until the material partly oxidizes. On experimentation it is found that a curve of hysteresis is obtained which has an approximately linear progress throughout a large zone of 60  $H$ , owing to which the permeability throughout this zone is relatively small but on the contrary the effective permeability throughout the same zone is large and practically constant. The linearity of the curve of hysteresis 65 also results in the effective permeability depending only slightly on the value of  $\Delta H$  and consequently on the alternating current amplitude. In addition, in contradistinction to the previously used material, this material has a small residual magnetism at a normal coercive force.

The explanation of these phenomena is due in all probability to the fact that owing to oxidation of the material microscopically small fissures are produced which act as air gaps and consequently bring about the typical progress of the curve of hysteresis.

The material produced by the process of 30 the invention is pre-eminently suitable for use as the core of a transformer or as some part of it, such as a lamella or a transformer sheet. Very good results have been obtained by subjecting to the process of the invention 85 an alloy of iron containing at least 40% of nickel.

If, for example, transformer-core-plates containing 50% nickel and approximately 0.095% carbon are heated in air at a temperature of about 900° C. during 15-20 minutes, the material thereafter still contains approximately 0.04% carbon. The heating operation however, should not be continued too long as otherwise the oxidation becomes too strong 95 and the magnetic properties grow weaker.

The invention will be more clearly understood by reference to the accompanying drawings. In these drawings:

Figure 1 is a comparative view of the 100

curves of hysteresis which are produced on testing a material which is only decarbonized, and a material which is worked by the process of the invention.

5 Figure 2 is a comparative view of the effective permeability at different values of  $H$  of the two curves of hysteresis shown in Figure 1.

10 Figure 3 is an enlarged view of the progress of  $\Delta B$  at cyclically varying  $\Delta H$ .

15 Figure 1 shows two curves of hysteresis, curve I of a material which is only decarbonized, curve II of a material which after decarbonization has been oxidized. In order that the characteristic properties of the curves should be well pronounced they will be compared at two values of the intensity of field  $H'$  and  $H''$ . By reason of alternating currents, cyclic variations  $\Delta H$  about the two 20 values  $H'$  and  $H''$  ensue. The variations  $\Delta B$  then measured show, graphically plotted, the progress as partly shown in Figure 1 and in Figure 3. To a maximum  $\Delta H$  corresponds a maximum  $\Delta B$ , the coefficient of both:

25 
$$\frac{\text{maximum } \Delta B}{\text{maximum } \Delta H},$$

30 or in other words the effective permeability, corresponds to the tangent of the angle made by the longitudinal axis of the loop with the  $H$ -axis (Figure 3). At the various values  $H'$  and  $H''$  this angle is found to be greatly different for curve I and little different for curve II. In Figure 3 are plotted the variations 35  $\Delta B$  at a large and at a small amplitude of  $\Delta H$ . The effective permeability is found to depend greatly in the curve I and slightly in the curve II on the amplitude of  $\Delta H$ .

40  $\alpha_1$  and  $\alpha_2$  designate the angles at various values of  $H$ . These angles are found to differ much more in curve I than in curve II.

45 In Figure 2 the various values of effective permeability are measured for any point of the curve of hysteresis and are plotted as a function of  $H$ . It is conspicuous from this graphic representation how the effective permeability in the case of the material I depends greatly and in the case of material II depends slightly on the intensity of field  $H$ .

50 What we claim is:

55 A transformer core comprising magnetic material which is substantially decarbonized and partly oxidized to such an extent that the hysteresis curve is substantially straight.

WIEBOLD FRANS BRANDSMA.  
POPKO REINDER DIJKSTERHUIS.  
GERARDUS JOHANNES SIZOO.  
GOTTFRIED BRUNO JONAS.